

## UNITED STATES PATENT OFFICE

2,322,982

## PHOTOGRAPHIC PRINTING MATERIAL

Gottlieb von Poser, Wiesbaden, Germany; vested  
in the Alien Property CustodianNo Drawing. Application January 4, 1941, Serial  
No. 373,139. In Germany December 27, 1939

15 Claims. (Cl. 95—7)

The present invention relates to a process of enhancing the light-sensitiveness of photographic printing material containing diazo-compounds.

It is already known that photographic printing materials can be obtained by means of light-sensitive diazo-compounds. Diazo-compounds which are suitable for such a process have to satisfy, as is known, a great number of requirements. Many diazo-compounds are known which in various respects are suitable for diazotype purposes, but nevertheless have not acquired any practical importance, since their light-sensitivity is too small.

The various colorless or only slightly colored diazo-compounds particularly belong to said kind of diazo-compounds. The afore-named diazo-compounds are in most cases distinguished by the fact that the photographic prints prepared therewith have only a slight tendency to turn yellow. Moreover, they are particularly suitable for the production of reflex copies. They yield reflex copies very rich in contrast. Furthermore the dyestuffs forming the picture of the reflex copies strongly absorb chemically active light if suitable azo-components are used as this is described in detail in the co-pending U. S. Patent Application Serial No. 276,420 filed May 29, 1939, now U. S. Patent No. 2,246,425 of June 17, 1941. The reflex copies are therefore well suited for being reproduced on photographic printing paper, for instance diazotype paper. In spite of these favorable properties the diazo-compounds in question have acquired only very little practical importance since their light-sensitivity is much smaller than that of the usual colored amino-diazo-compounds and diazo-anhydrides. In comparison with the latter they require an exposure to light which, for instance, is three to ten times as long as even longer.

The terms "relatively light insensitive diazo-compound" or "diazo-compound of small light-sensitivity" respectively in the following description and the claims mean diazo-compounds the light sensitiveness of which is at most about a half of that of the 1-diazo-4-dimethylaniline provided that a usual source of light, for instance the arc lamp is employed for the exposure. Also as used herein the term "quinones" means aromatic keto compounds containing the quinone grouping such as anthraquinone and its derivatives, benzanthrone, naphthoquinone, naphthanthraquinone, and diphenolbenzoquinone; the term "phenones" means aromatic keto compounds wherein the keto group is a bridge member, but not a part of a ring system such as benzophenone

and its derivatives, the term "fluorenones" means fluorenone and its derivatives; and the term "acridones" means acridone and its derivatives.

Now I have found that the light-sensitivity of relatively light-insensitive diazo-compounds may be enhanced when they are combined with aromatic keto-compounds, particularly such as are soluble in water or in a mixture of water and alcohol respectively. Preferably the said keto-compounds should contain more than one aromatic nucleus, for example two or three aromatic nuclei. Keto-compounds which contain a CO-group in a benzene ring or another ring, for instance quinones have proven particularly good. However, also compounds of the benzophenone type are also suitable. It is furthermore desirable that the sensitizers be not dyestuffs. They should preferably be colorless or only slightly colored.

Suitable sensitizers are for instance anthraquinone and the derivatives thereof. Such derivatives are especially useful as are readily soluble in water. They may be added to the aqueous or aqueous-alcoholic solutions containing the diazo-compounds on producing the photographic printing materials. The benzene nuclei of the anthraquinone may carry, for instance, simple substituents, such as alkyl groups, halogen atoms, carboxylic or sulfonic acid groups. Anthraquinone sulfonic acids or the alkali metal salts thereof are particularly suitable. Above all 2,7-anthraquinone-disulfonic acid must be mentioned. Beta-anthraquinone-mono-sulfonic acid may also be used with good success. Instead of the anthraquinone or its derivatives there may be used the benzanthrone or the derivatives thereof, especially the benzanthrone-sulfonic acids. The 2,5-dipheno-1,4-benzoquinone is likewise suitable, especially in the form of sulfonic acid or the sodium salt of sulfonic acid.



Furthermore, there may for instance be used the 1,2-naphthoquinone-4-sulfonic acid and the fluorenone-2,7-disulfonic acid. Other suitable sensitizers are the sulfonation product of the acridone (produced by introducing acridone into ten times its weight of sulfuric acid monohydrate, heating the whole for 1 hour on the vapor bath, and precipitating it by the addition of ice water),

the sulfonation product of naphthanthaquinone (produced by introducing naphthanthaquinone into ten times its weight of fuming sulfuric acid containing 20 per cent of free  $\text{SO}_3$  and heating the whole for half an hour on the vapor bath). The sulfonation products of benzophenone or of para-chloro-benzophenone are likewise useful. These products may be obtained by heating benzophenone or para-chloro-benzophenone with six times its weight of fuming sulfuric acid containing 20 per cent of free  $\text{SO}_3$  to 90° C., adding once its weight of fuming sulfuric acid of 70 per cent  $\text{SO}_3$  and further heating the whole for  $\frac{1}{4}$  hour. The sodium salts of the above-named sulfonation products may be separated from the solutions by the addition of ice-water and caustic soda.

By means of the afore-named sensitizers the light-sensitiveness of relatively light-insensitive diazo-compounds may be enhanced to a multiple so that they then satisfy the practical requirements. Colorless diazo-compounds of the benzene series which are free from amino groups may be sensitized with particularly good success, for example diazo phenols and diazo phenol ethers. Diazo phenol alkyl ethers i. e. the diazotization products of p-anisidine, o-anisidine and similar alkyl ethers of amino-phenols are particularly well suitable for the purpose of the invention. Other suitable colorless diazo compounds are mentioned in the copending application 276,420. Slightly colored compounds, for instance the tetrazotized dianisidine, may, likewise be sensitized.

The proportion of the sensitizers present in the photographic printing material may be just as large as that of the diazo compounds. In general, however, an effect may be produced by an essentially smaller quantity of the sensitizer than that named above. In many cases a few percentages calculated on the diazo-compound are sufficient. But within certain limits there exists a proportionality between the enhancement of the light-sensitiveness and the quantity of the sensitizers added. Additions usual in diazo-type-processes may be given to the solutions. If colorless diazo compounds are used, it is advisable to add bleaching-out dyestuffs to the solutions; the process of exposure to light may thus be well observed. The usual supports, such as paper and films of all kinds may be used. If films are applied, the sensitizing effect is in general manifested particularly well.

The following examples serve to illustrate the invention, but they are not intended to limit it thereto:

(1) A foil of regenerated cellulose is bathed in a solution containing in 1000 cc. of water

|                                         | Grams |
|-----------------------------------------|-------|
| 5-chloro-2-diazobenzene-1-sulfonic acid | 10    |
| Tartaric acid                           | 12    |
| Boric acid                              | 6     |
| Sodium naphthalene-1,3,6-trisulfonate   | 20    |
| Sodium 2-naphthol-3,6-disulfonate       | 8     |
| Sodium anthraquinone-2,7-disulfonate    | 5     |

By exposing the dried film for about 1 minute to the light of an arc lamp (18 amperes, distance=40 cm.) under an original and developing it by the treatment with ammonia gas, an orange-red image is obtained. By preparing the film with the same solution while omitting the anthraquinone derivative, 6-7 minutes would be required for copying the original.

(2) A cellulose-hydrate foil is impregnated with a solution containing in 1000 cc. of water

|                                         | Grams |
|-----------------------------------------|-------|
| 5-ethoxy-2-diazobenzene-1-sulfonic acid | 10    |
| Tartaric acid                           | 15    |
| Boric acid                              | 8     |
| Sodium 2-naphthol-3,6-disulfonate       | 10    |
| Sodium 2,7-anthraquinone-disulfonate    | 20    |

10 With the aid of the film thus prepared diazo photographic printing copies may be produced in the usual manner. The light-sensitiveness of the film amounts to about 15 times the light-sensitiveness of a copying material prepared in the same manner, but without the addition of the anthraquinone-compound.

Instead of the afore-named diazo-compound there may be used with a similar success the 4-diazo-1-anisole, the 2-diazo-1-anisole, the 4-diazo-1-phenol, the 2-diazo-5-hydroxybenzene-1-sulfonic acid and the 4-diazo-1-phenoxybenzene.

(3) An acetyl-cellulose film superficially saponified is coated with a solution containing in 1000 cc. of water

|                                                           | Grams |
|-----------------------------------------------------------|-------|
| Beta - naphthalene - diazonium - fluoro - boric acid salt | 60    |
| Tartaric acid                                             | 80    |
| Boric acid                                                | 60    |
| Sodium 2-naphthol-3,6-disulfonate                         | 30    |
| Sodium anthraquinone-2,7-disulfonate                      | 30    |

The exposure to light of the copying material obtained amounts to less than the fourth part of the exposure to light required by the corresponding material which has been prepared without the anthraquinone-compound.

(4) A diazo photographic printing material is obtained by coating photographic crude paper with a solution containing in 1000 cc. of water

|                                          | Grams |
|------------------------------------------|-------|
| 5-hydroxy-2-diazobenzene-1-sulfonic acid | 20    |
| Tartaric acid                            | 20    |
| Boric acid                               | 10    |
| 45 Resorcine                             | 15    |
| Sodium anthraquinone-2,7-disulfonate     | 20    |

(5) A photographic printing foil is produced by saturating a foil of regenerated cellulose with a solution containing in 1000 cc. of water

|                                      | Grams |
|--------------------------------------|-------|
| 2-acetylamino-5-diazo-1-benzoic acid | 15    |
| Tartaric acid                        | 20    |
| Naphthalene-1,3,6-trisulfonic acid   | 60    |
| 55 Sodium 2-naphthol-3,6-disulfonate | 8     |
| Sodium anthraquinone-2,7-disulfonate | 5     |

(6) A photographic crude paper is coated with a solution containing in 1000 cc. of water

|                                                                         | Grams |
|-------------------------------------------------------------------------|-------|
| Zinc chloride double salt of 2,4-dimethoxy-benzene-1-diazonium chloride | 12    |
| Sodium anthraquinone-1,5-disulfonate                                    | 2     |

65 With the help of the photographic printing material thus produced diazotypes may be prepared which are developed in known manner according to the method of moist developing.

I claim:

70 1. Light-sensitive material which consists of a carrier having a layer comprising a diazo-compound of small light-sensitiveness and a sensitizer consisting in an aromatic keto-compound selected from the group consisting of quinones, phenones, acridones and fluorenones.

2. Light-sensitive material according to claim 1 wherein the said sensitizer is water soluble.
3. Light sensitive material which consists of a carrier having a layer comprising a diazo compound of small light-sensitiveness and as a sensitizer a water soluble, substantially colorless anthraquinone compound.
4. Light-sensitive material which consists of a carrier having a layer comprising a substantially colorless diazo-compound of small light-sensitiveness and a sensitizer consisting in an aromatic keto-compound selected from the group consisting of quinones, phenones, acridones and fluorenones.
5. Light-sensitive material according to claim 4 wherein the said sensitizer is water soluble.
6. Light-sensitive material which consists of a carrier having a layer comprising a substantially colorless diazo compound of small light-sensitiveness and as a sensitizer a water soluble, substantially colorless anthraquinone compound.
7. Light-sensitive material which consists of a carrier having a layer comprising a substantially colorless diazo phenol ether of small light-sensitiveness and a sensitizer consisting in an aromatic keto-compound selected from the group consisting of quinones, phenones, acridones and fluorenones.
8. Light-sensitive material according to claim 7 wherein the said sensitizer is water soluble.
9. Light-sensitive material which consists of a carrier having a layer comprising a substantially colorless diazo phenol ether of small light-sensi-
- tiveness and as a sensitizer a water soluble, substantially colorless anthraquinone compound.
10. Light-sensitive material which consists of a carrier having a layer comprising a substantially colorless diazo phenol alkyl ether of small light-sensitiveness and a sensitizer consisting in an aromatic keto-compound selected from the group consisting of quinones, phenones, acridones and fluorenones.
11. Light-sensitive material according to claim 10 wherein the said sensitizer is water soluble.
12. Light-sensitive material which consists of a carrier having a layer comprising a substantially colorless diazo phenol alkyl ether of small light-sensitiveness and as a sensitizer a water soluble, substantially colorless anthraquinone compound.
13. Light-sensitive material which consists of a carrier having a layer comprising a substantially colorless diazo phenol alkyl ether of small light-sensitiveness and as a sensitizer the 2,7-anthraquinone disulfonic acid.
14. Light-sensitive material which consists of a carrier having a layer comprising a substantially colorless diazo phenol alkyl ether of small light-sensitiveness and as a sensitizer the 2-anthraquinone sulfonic acid.
15. Light-sensitive material which consists of a carrier having a layer comprising a substantially colorless diazo phenol alkyl ether of small light-sensitiveness and as a sensitizer the 1,4-dichloro-2-anthraquinone sulfonic acid.

GOTTLIEB VON POSER.